

[54] PROCESS FOR PRODUCING AN  
ENAMELLING STEEL SHEET

[75] Inventors: **Hisashi Gondo; Hiroshi Takechi; Kazuo Namba, all of Kisarazu; Matsuo Usuda; Kouichi Kawasaki, both of Kimitsu, all of Japan**

[73] Assignee: **Nippon Steel Corporation, Tokyo, Japan**

[22] Filed: **Mar. 7, 1974**

[21] Appl. No.: **448,958**

## [30] Foreign Application Priority Data

Mar. 9, 1973 Japan..... 48-27169

[52] U.S. Cl..... 148/2; 148/12 C; 75/123

[51] Int. Cl. .... C21D 7/02; C21D 7/13; C21D 9/46

[58] Field of Search ..... 148/12 C, 12 F, 2; 75/123 E

## [56] References Cited

## UNITED STATES PATENTS

|           |        |                                |
|-----------|--------|--------------------------------|
| 3,666,452 | 5/1972 | Korchynsky et al..... 148/12 F |
| 3,666,570 | 5/1972 | Korchynsky et al..... 148/12 F |
| 3,671,336 | 6/1972 | Korchynsky et al..... 148/12 F |

## FOREIGN PATENTS OR APPLICATIONS

1,192,794 5/1970 United Kingdom

Primary Examiner—W. Stallard  
Attorney, Agent, or Firm—Toren, McGeady and Stanger

## [57] ABSTRACT

A process for producing an enamelling steel sheet which comprises tapping molten steel with manganese content not more than 0.40%, lowering the carbon content in the molten steel to not more than 0.01%, adding titanium to the molten steel in an amount enough to obtain a titanium content between 0.01 and 0.3%, preferably between 0.03 and 0.1%, and also adding one or more of rare earth elements such as lanthanum, cerium, neodymium, praseodymium, and samarium (hereinafter called Rem) in total amount between 0.01 and 0.15%, preferably 0.02 and 0.12%, casting the molten steel into ingot or slab, hot rolling and then cold rolling the ingot or slab preferably at a cold rolling rate between 30 and 90% and then annealing the steel sheet.

12 Claims, 1 Drawing Figure

Thickness of Initial  
Solidified Layer ( $\mu$ )





## PROCESS FOR PRODUCING AN ENAMELLING STEEL SHEET

The present invention relates to a process for producing an enamelling steel sheet having remarkable resistance against "fish-scale" as well as good non-aging property and deep-drawability and yet showing large weight decrease by acid pickling.

It is required for an enamelling steel sheet that it is free from the surface defect due to hydrogen, namely, "fish-scale", and it has good adhesion to enamelling glaze. At the same time, the enamelling steel sheet is required to have good workability such as deep-drawing because the enamelling steel sheet is very often subjected to severe forming into bath tubs, tableware, sanitary utensiles and so on and then enamelled. It is also required in case of single application of enamelling glaze that the enamelling steel sheet is free from surface defects due to carbonaceous gas, such as foams and blisters as well as free from the strain due to enamel firing and that it has a large acid pickling rate from the point of productivity.

In order to meet the above requirements, it has been conventionally known that titanium is added to the steel to fix carbon and nitrogen in the steel so as to render the steel non-aging and to improve resistance against the fish-scale by the titanium content in the steel. In this case, however, the amount of titanium to be added to fix the carbon increases, the steel hardens and the production cost increases. Thus, in order to eliminate these defects, it has been conventionally practised to lower the carbon and oxygen contents in the steel preliminary by vacuum degassing, or to maintain the ratio of titanium to carbon of  $Ti/C \geq 10$  so as to improve deep-drawability.

The steel sheet produced by the above conventional methods, however, has a defect that surface defects due to titanium compounds appear on the steel surface in some cases, thus causing lowering of the production yield. Also in case where titanium is added to the steel, the weight decreases during the acid pickling treatment conducted as a preliminary treatment for the enamel firing is relatively small so that the time required for the preliminary treatment is necessitated to be longer in case of the single application of enamelling glaze. This is undesirable from the point of the productivity.

Therefore, one of the objects of the present invention is to provide a process for producing an enamelling steel sheet having remarkably excellent resistance against the fish-scale and free from the above defects.

The features of the present invention are summarized as under.

1. A process for producing an enamelling steel sheet which comprises tapping molten steel with manganese content not more than 0.40%, lowering the carbon content in the molten steel to not more than 0.01%, adding titanium to the molten steel in an amount enough to obtain a titanium content between 0.01 and 0.3%, preferably between 0.03 and 0.1%, and also adding one or more of rare earth elements such as lanthanum, cerium, neodymium, praseodymium, and samarium (hereinafter called Rem) in total amount between 0.01 and 0.15%, preferably 0.02 and 0.12%, casting the molten steel into ingot or slab, hot rolling and then cold rolling the ingot or slab preferably at a cold rolling rate between 30 and 90% and then annealing the steel sheet.

2. A process for producing an enamelling steel sheet which comprises tapping molten steel with a manganese content not more than 0.40%, lowering the carbon content in the molten steel to not more than 0.01% by vacuum degassing, adding Rem to the steel in a total amount between 0.01 and 0.15%, preferably 0.02 and 0.12% prior to or at the same time of casting the steel into an ingot mold, leaving the steel after casting into the mold until an initial solidified layer is formed, adding titanium to the non-solidified portion so as to obtain titanium content between 0.01 and 0.3%, preferably 0.03 and 0.1%, hot rolling and cold rolling and annealing the steel sheet.

3. A process for producing an enamelling steel sheet which comprises tapping molten steel with a manganese content not more than 0.40%, lowering the carbon content in the steel to not more than 0.01% by vacuum degassing, leaving the steel after casting to ingot mold until an initial solidified layer is formed, adding titanium and Rem to the non-solidified portion in an amount to obtain a titanium content between 0.01 and 0.3%, preferably 0.03 and 0.1%, and a total content of Rem between 0.01 and 0.15%, preferably between 0.02 and 0.12%, casting the steel into ingot, hot rolling and cold rolling the steel preferably with a cold rolling reduction rate between 30 and 90%, and then annealing the steel sheet.

The present invention will be described in more details referring to the attached drawings.

FIG. 1 shows the initial solidified layer thickness of the steel sheet (A) produced according to the present invention.

For the production of the steel according to the present invention, the molten steel is tapped with a manganese content not more than 0.40%. A smaller manganese content is desirable for reducing the strain due to the enamel firing as well as from the point of material quality, and thus its upper limit is defined as 0.40%. Then, the molten steel is subjected to vacuum degassing treatment to lower the carbon content to not more than 0.01%. The reason for limiting the carbon content to not more than 0.01% is to prevent occurrence of the surface defects such as foams and blisters due to the carbonaceous gas and to prevent the strain due to the enamel firing. The oxygen content is also reduced by the degassing, but the remaining oxygen can be further reduced by a preliminary deoxydation with aluminum, for example, after the completion of the degassing treatment, if necessary.

Prior to the pouring the molten steel into the ingot mold or during the pouring, titanium and Rem are added to the molten steel so as to obtain a titanium content between 0.01 and 0.30%, preferably 0.03 and 0.10% and a total Rem content between 0.01 and 0.15%, preferably 0.03 and 0.12%. The reason for limiting the titanium content in the steel between 0.01 and 0.30%, preferably 0.03 and 0.10% is that if the titanium content is more than 0.30%, the steel hardens and press formability is lowered and the production cost increases, while the titanium content is less than 0.01%, no substantial improvement on the resistance against the fish-scale and deep-drawability can be expected. Meanwhile the reason for limiting the Rem content between 0.01 and 0.15%, preferably 0.02 and 0.12% is that a Rem content more than 0.15% will cause increased production cost and, on the other hand, a Rem content less than 0.01% no substantial improvement on the resistance against the fish-scale

can be expected.

The steel slab produced according to the present invention is subjected to hot rolling, acid pickling, electrical cleaning, annealing and, if necessary, temper rolling. The hot rolling may be conducted under ordinary conditions, but desirable results can be obtained by conducting the hot rolling with coiling temperature between 450° and 800°C, preferably 550° and 730°C. If the hot coiling temperature exceeds 800°C, it is difficult to adjust the temperature, and on the other hand if the coiling temperature is lower than 450°C the improvement effect of the resistance against the fish-scale is reduced.

Regarding the cold rolling, a reduction rate not less than 30% is desirable for obtaining desirable material quality, but with a reduction rate more than 90% the required thickness of the hot rolled steel sheet is too thick for practical use. On the other hand, with a reduction rate less than 30%, desired deep-drawability can not be obtained.

The annealing may be done by any of a box annealing, a continuous annealing and other annealing methods, and the annealing temperature should be between 650° and 1000°C, preferably between 650° and 910°C in case of the box annealing and an open coil annealing, and between 700° and 980°C in case of the continuous annealing. If the annealing temperature is lower than the lower limit, softening of the steel caused by recrystallization is not enough so that desirable workability is not obtained. On the other hand, if the temperature is higher than the upper limit, the amount of transformation into austenite is large so that good deep-drawability can not be obtained, and the higher temperature is not desirable also from the point of the economy of the furnace.

The resistance against the fish-scale of the steel sheet produced according to the present invention defined in paragraph (1) hereinbefore is remarkably good, and it has been found that much larger effect can be obtained as compared with the total combining effect obtained by addition of titanium alone, and effect obtained by addition of Rem alone.

The present inventors have conducted further extensive studies and experiments for solving the problems such as the occurrence of the surface defects due to the titanium compounds and the lowering of the weight decrease during the acid pickling, and have found that these problems can be solved by forming an initial solidified layer containing no titanium on the steel 50 surface according to the present invention as defined in the paragraphs (2) and (3) as hereinbefore stated.

Embodiments of the present invention as defined in the paragraphs (2) and (3) will be described under.

The present invention of the paragraph (2) may be 55 conducted as under.

Molten steel containing not more than 0.40% of manganese preferably not more than 0.25% of manganese is tapped, and subjected to vacuum degassing to reduce the carbon content to less than 0.01%, and then prior to or at the same time of pouring the molten steel into an ingot mold, Rem is added so as to obtain a total Rem content between 0.01 and 0.15%, preferably 0.02 and 0.12%, and the steel is left after the pouring into the mold until an initial solidified layer is formed, and titanium is added to the non-solidified portion so as to obtain a titanium content between 0.01 and 0.3%, preferably 0.03 and 0.10%.

Rem may be added together with titanium to the non-solidified portion of the ingot after the molten steel is cast into the mold and the initial solidified layer containing no titanium and Rem is formed according to the present invention defined in the paragraph (3).

Namely, molten steel with a manganese content not more than 0.40%, preferably not more than 0.25% is tapped and subjected to vacuum degassing treatment to lower the carbon content to not more than 0.01%, and the molten steel is left after it is cast into the mold until an initial solidified layer is formed, and then titanium and Rem are added to the non-solidified portion so as to obtain a titanium content between 0.01 and 0.3%, preferably 0.03 and 0.1%, and a total Rem content between 0.01 and 0.15%, preferably 0.02 and 0.12%.

The initial solidified layer produced by the present invention as defined in the paragraphs (2) and (3) is different from the conventional rim layer formed by the rimming action in their formation mechanisms, and it is 20 the important difference that the initial solidified layer is formed without rimming action, and thus the surface of the ingot produced by the present invention is as good as that of the rimmed steel. Further as the initial solidified layer of the steel produced by the present invention does not contain titanium, surface defects due to the titanium compounds are not caused at all, and the cold rolled steel sheets produced according to the present invention do not contain titanium in their surface layer and thus their weight decrease in acid 25 pickling is large enough so that the time required by the acid pickling treatment is largely reduced. When Rem is added in the ladle as in the paragraph (2) of the present invention, good uniformity of the Rem addition in the steel is assured, and in case of the paragraph (3) of the present invention, a remarkably good yield of Rem is assured.

Examples of the present invention will be described hereinunder.

Molten steel prepared in a converter, having a ladle analysis showing 0.018% of carbon and 0.17% of manganese was subjected to vacuum degassing and pre-deoxidized by addition of aluminum. In case of the steel A, the molten steel was left one minute after casting into an ingot mold to form an initial solidified layer in the ingot, and titanium and Rem were added to the non-solidified portion. In case of the steel B, Rem was added simultaneously when the ingot-casting of the molten steel was started, and the molten steel was left 1 minute after the casting to form an initial solidified layer, and titanium was added to the non-solidified portion. In case of the steel C, titanium and Rem were added simultaneously when the ingot-casting was started.

In case of the comparative steels D and E, the molten steel was left one minute after the ingot-casting to form an initial solidified layer in the steel ingot, and titanium was added to the non-solidified layer (steel D) and Rem was added to the non-solidified layer (steel E). All of the inventive steels A, B, and C and the comparative steels D and E were hot rolled to 6.5mm thickness with a hot coiling temperature of 590°C, cold rolled to 2.0mm thickness, and subjected to a box annealing at 700°C for 12 hours and 1% temper rolling.

The chemical analyses of the steel sheets thus produced are shown in Table 1 and the mechanical properties are shown in Table 2. The thickness of the initial solidified layer of the inventive steel A is shown in FIG. 1. As understood from Table 2, the inventive steels A,

B, and C show excellent deep-drawability but does not show aging at all. Also these steel sheets were subjected to enamel firing with single application of glaze using glaze which easily causes fish-scale, and fish-scale occurrence was investigated.

It has been confirmed from the results shown in Table 4 that the inventive steels A, B, and C show far better resistance against the occurrence of fish-scale as compared with the comparative steel D in which only titanium is added and the steel E in which only Rem is added. This remarkable results are obtained by the combined addition of titanium and Rem, and it has

10 having the initial solidified layer had appearance as good as that of a rimmed steel and was completely free from surface defects.

Further, when enamel glaze was applied twice and fired, the inventive steels showed always excellent fish-scale resistance and other enamelling qualities. The inventive steel may be enamelled as hot-rolled condition without any disadvantage, and the inventive steels give remarkable industrial advantages when they are applied to hot dipping, electrolytic zinc-plating, tin-plating, copper-plating and aluminium-plating as they show good adhesion thereto.

Table 1.

| Chemical Analysis of Steel Sheets (% by weight) |   |       |      |      |       |       |        |          |           |       |        |                                                |
|-------------------------------------------------|---|-------|------|------|-------|-------|--------|----------|-----------|-------|--------|------------------------------------------------|
|                                                 |   | C     | Mn   | Si   | P     | S     | O      | Total Ti | Total Rem | Ce    | N      | Remarks                                        |
| Inventive                                       | A | 0.004 | 0.17 | 0.02 | 0.011 | 0.005 | 0.0030 | 0.049    | 0.105     | 0.030 | 0.0069 | with initial solidified layer                  |
| Inventive                                       | B | 0.004 | 0.17 | 0.02 | 0.012 | 0.006 | 0.0020 | 0.043    | 0.095     | 0.035 | 0.0070 | (Rem is contained in initial solidified layer) |
| Inventive                                       | C | 0.004 | 0.17 | 0.02 | 0.011 | 0.007 | 0.0040 | 0.048    | 0.115     | 0.052 | 0.0066 | with no initial solidified layer               |
| Comparative                                     | D | 0.005 | 0.18 | 0.02 | 0.011 | 0.009 | 0.0030 | 0.046    | —         | —     | 0.0060 | with initial solidified layer                  |
| Comparative                                     | E | 0.003 | 0.17 | 0.02 | 0.011 | 0.007 | 0.0050 | —        | 0.093     | 0.038 | 0.0086 | "                                              |

Table 2:

| Mechanical Properties of Steel Sheet<br>(2.0mm thickness) |    |      |      |    |      |                                                        |
|-----------------------------------------------------------|----|------|------|----|------|--------------------------------------------------------|
|                                                           | YP | TS   | EI   | T  | n    | Yield point elongation<br>100°C × 60 minutes aging (%) |
| Inventive                                                 | A  | 16.0 | 28.8 | 55 | 1.95 | 0.26                                                   |
| Inventive                                                 | B  | 16.2 | 28.1 | 56 | 1.90 | 0.26                                                   |
| Inventive                                                 | C  | 15.3 | 28.2 | 54 | 1.80 | 0.26                                                   |
| Comparative                                               | D  | 13.4 | 29.8 | 54 | 1.92 | 0.26                                                   |
| Comparative                                               | E  | 23.4 | 30.8 | 54 | 1.36 | 0.21                                                   |

been discovered through various studies that same or similar results can not be obtained if titanium and other inclusions are present simultaneously. As another method for determining the fish-scale resistance, measurements were made on hydrogen permeation times. According to this method, electrolysis was effected on one side of the steel sheet, and the time required by hydrogen for diffusing the steel sheet and reaching the other side of the steel sheet (this time called the hydrogen permeation time) was measured. As longer hydrogen permeation time represents larger ability of absorbing hydrogen within the steel sheet, and therefore better fish-scale resistance. The results of measurements at 25°C of the hydrogen permeation times of the steels A, B, C, D and E according to the method are shown in Table 5, from which it is clear that the inventive steels A, B and C show a remarkably long hydrogen permeation time. It has been also confirmed that the inventive steels A, B, and C were completely free from defects such as foams and blisters after the enamel firing with single application of glaze, and showed very good adhesion.

Next, the inventive steels A, B, and C were immersed in 10%  $H_2SO_4$  solution at 70°C for 10 minutes and measured for weight decrease by acid pickling. The results are shown in Table 3. The inventive steels A and B showed a remarkably large weight decrease and were found to be very advantageous for efficiency of enamel firing. Also the surface of the inventive steels A and B

Table 3.

|                 | Weight decrease by acid pickling (mg/dm <sup>2</sup> ) |
|-----------------|--------------------------------------------------------|
| Inventive Steel |                                                        |
| A               | 680                                                    |
| B               | 675                                                    |
| C               | 342                                                    |

Table 4.

|                   | Fish-scale occurrence (%) |
|-------------------|---------------------------|
| Inventive Steel   |                           |
| A                 | 0                         |
| B                 | 0                         |
| C                 | 0                         |
| Comparative Steel |                           |
| D                 | 32                        |
| E                 | 40                        |

Table 5

| Inventive Steel   | Hydrogen Permeation Time (min.) |
|-------------------|---------------------------------|
| A                 | 168                             |
| B                 | 147                             |
| C                 | 180                             |
| Comparative Steel |                                 |
| D                 | 24.5                            |
| E                 | 52                              |

What is claimed is:

1. A process for producing an enamelling steel sheet which comprises tapping molten steel with a manganese content of not more than 0.40%, lowering the carbon content in the molten steel to not more than 0.01%, adding titanium to the molten steel in an amount enough to obtain a titanium content between 0.01 and 0.3%, and adding one or more elements selected from the group consisting of the rare earth elements in a total amount between 0.01 and 0.15%, casting the molten steel into ingot or slab, hot rolling and then cold rolling the ingot or slab and then annealing the steel sheet.

2. The process of claim 1 wherein the amount of titanium is between 0.03 and 0.1%.

3. The process of claim 1 wherein the rare earth element is lanthanum, cerium, neodymium, praseodymium or samarium.

4. The process of claim 1 wherein the amount of rare earth element is between 0.02 and 0.12%.

5. The process of claim 1 wherein the cold rolling rate is between 30 and 90%.

6. A process for producing an enamelling steel sheet which comprises tapping molten steel with a manganese content of not more than 0.40%, lowering the carbon content in the molten steel to not more than 0.01% by vacuum degassing, adding one or more elements selected from the group consisting of the rare earth elements to the steel in a total amount between 0.01 and 0.15%, prior to or at the same time of casting

the steel into an ingot mold, leaving the steel after casting in the mold until an initial solidified layer is formed, adding titanium to the non-solidified portion so as to obtain a titanium content between 0.01 and 0.3%, and hot rolling, cold rolling and annealing the steel sheet.

7. The process of claim 6, wherein the amount of rare earth element is between 0.02 and 0.12%.

8. The process of claim 6, wherein the amount of titanium is between 0.03 and 0.1%.

9. A process for producing an enamelling steel sheet which comprises tapping molten steel with a manganese content of not more than 0.40%, lowering the carbon content in the steel to not more than 0.01% by vacuum degassing, leaving the steel after casting in an ingot mold until an initial solidified layer is formed, adding titanium and an element selected from the group consisting of one or more of the rare earth elements to the non-solidified portion in an amount to obtain a titanium content between 0.01 and 0.3%, and a total content of the rare earth elements between 0.01 and 0.15%, casting the steel into an ingot, hot rolling and cold rolling the steel, and then annealing the steel sheet.

10. The process of claim 9, wherein the amount of titanium is between 0.03 and 0.1%.

11. The process of claim 9, wherein the amount of rare earth element is between 0.02 and 0.12%.

12. The process of claim 9, wherein the cold rolling rate is between 30 and 90%.

\* \* \* \* \*